

Feb. 2, 1937.

G. ANDERSEN

2,069,469

PROCESS FOR THE PRODUCTION OF METALS AND ALLOYS  
WITH VERY SMALL CONTENTS OF CARBON  
Filed Dec. 22, 1933

Fig.1.



Fig.2.



## UNITED STATES PATENT OFFICE

2,069,469

PROCESS FOR THE PRODUCTION OF  
METALS AND ALLOYS WITH VERY  
SMALL CONTENTS OF CARBON

Gustav Andersen, Copenhagen, Denmark

Application December 22, 1933, Serial No. 703,641  
In Norway December 31, 1932

3 Claims. (Cl. 75—133)

This invention relates to a process for the production of metals and alloys with very small contents of carbon.

It is known that very important difficulties are met in the production of metals and alloys with very small contents of carbon, for instance chromium and manganese with very small contents of carbon as well as their alloys, especially chrome- or manganese-iron and steel alloys, due 10 to the fact that the said metals possess a great affinity for carbon.

As a rule, the production of stainless steel, for instance, is realized by using an alloy of chromium and iron, having a high chromium content but a low content of carbon, which alloy is added 15 to the finished, melted steel.

Obviously, the indirect producing processes are very expensive, on the one hand due to difficulty of making such a chrome-iron alloy and on 20 the other hand due to the losses arising from the melting together, and accordingly it is better to use a direct process in which a direct reduction of the alloy metals in the main metal is effected. In one of said processes, bricks of chromite 25 thoroughly ground are added, with ferro-silicon or with a silicon containing reducing means, to melted and overheated iron. The additional metal in the alloy is reduced in the bath of metal which is thoroughly stirred, a direct production 30 of the alloy being thus effected, having the desired analysis, for instance a stainless steel.

Very often a process is used in which no carbon-containing reducing means are used, and in 35 which electrodes are used that are not allowed to come into direct contact with the metal for reduction purposes, but it is clear that an alloy will be obtained having a variable and too high a content of carbon. This process is especially suitable for high carbon contents. Apparently, 40 in the above process, the carbon which is absorbed comes from the raw materials, ore, ferro-silicon or slag.

Analyses made with the ore used show that it 45 has a carbon content of 0.04 to 0.10% or even more. In a further process ferro-silicon and limestone are used. Carbon is likely to be found in the foreign matters, plant fibers, leaves, earth, etc. getting mixed with the ore in the course of transportation or in ore bunkers.

50 An output of more than 60 to 70% of the

metal cannot be obtained, and most of the carbon present in ore, in reducing means or in slag will be found in the melted metal. For the above mentioned reason it will be understood that the final metal will always have a high carbon content, and on the other hand this carbon content is variable over wide limits.

The above drawbacks are eliminated in the process described here:

Before a charge of correctly determined quantities of ore, ferro-silicon or other silicon containing reduction means and limestone is put into an overheated main-metal bath, which only contains a very small quantity of carbon, it is submitted to a pre-treatment by heating it to a temperature of 1000° to 1100° C. i. e. without melting it in a strongly oxidizing flame, in order to burn out the carbon which is in the charge, and to have the limestone transformed into caustic lime.

The drawing shows diagrammatically how the process is practiced. Fig. 1 is a vertical section taken on the line I—I of Fig. 2 of a furnace adapted to the purpose. Fig. 2 is a horizontal view of the same furnace.

The charge is ground to a suitable size of grain (like grits or even smaller) thoroughly stirred up and loaded through a feeder 1 in a thin layer (about 4" thick) over a continuously rotating heating platform 2 where it will meet 30 the combustion gases from a hot strongly oxidizing flame 3 in countercurrent, the furnace being for instance of the type described in the U. S. A. patent application Ser. No. 703,640 of 1933.

After the treatment, the hot charge is discharged at 4 into closed iron boxes 5 for cooling and storing purposes.

If the combustion gases are to be used again in the process for heating purposes, the carbon dioxide is previously separated, for instance by 40 directing the gases which are conducted up through the feeder 1 through a caustic potash filter 6 or similar product before the gases are conducted back by a fan 7 to the furnace at the point where the oxidizing flame 3 is produced. 45 This purification by which sulphur is also eliminated, is very important if good results are to be obtained. Similarly it is necessary to use a strong oxidizing flame.

The charge which has been freed from carbon, 50

may be added directly to melted metal for a final high-temperature treatment, for instance to an iron bath having a very low carbon content. The determined quantity of charge is poured into 5 the iron bath directly from the closed box 8 in which it is stored in order to prevent its oxidation. Thus a metal having the precise, desired analysis is obtained.

Having thus described my invention what I 10 claim is:

1. A process for the production of metals and alloys with a very small content of carbon, by direct reduction of ore with silicon-containing reduction means on an over-heated metal bath 15 with a very small content of carbon, the said method including the use of a charge consisting of ore, limestone and silicon-containing reduc-

tion means, submitted, before being charged into the main metal bath, to a pre-treatment by heating it to 1000 to 1100° C. in a highly oxidizing flame whereby all the carbon is burnt away and the limestone is converted into burnt lime. 5

2. A process according to claim 1 including the crushing of the charge material in pieces of appropriate size and its mixing and spreading in a relatively thin layer on a continuously rotating heating platform, on which it is moved in counter-current to the direction of the highly oxidizing flame. 10

3. A process according to claim 1 including subsequent step of cooling the pre-treated charge material in a closed chamber and protecting the 15 said material against contamination.

GUSTAV ANDERSEN.